

# UNITED STATES PATENT OFFICE.

WERNER VON BOLTON, OF CHARLOTTENBURG, GERMANY, ASSIGNOR TO  
SIEMENS & HALSKE AKTIENGESELLSCHAFT, OF BERLIN, GERMANY.

## HOMOGENEOUS BODY OF HIGHLY-REFRACTORY METALS.

No. 817,783.

Specification of Letters Patent.

Patented April 10, 1906.

Original application filed January 5, 1904, Serial No. 187,830. Divided and this application filed September 29, 1905. Serial No. 280,639.

*To all whom it may concern:*

Be it known that I, WERNER VON BOLTON, a subject of the German Emperor, residing at Charlottenburg, near Berlin, Germany, 5 have made a new and useful Invention in Homogeneous Bodies of Highly-Refraactory Metals, of which the following is a specification.

My invention is directed particularly to a 10 homogeneous body of highly-refraactory metal, such as tantalum, which has a fusing-point at above 2,000° Celsius; and it has for its object to provide a metal of this nature which shall be ductile or capable of being rolled into thin 15 sheets or rolled or drawn into wires or rods.

Prior to my invention, so far as I am aware, there did not exist a relatively pure metal of a highly-refraactory type, such as tantalum, which was ductile or capable of being rolled 20 or drawn, and such a product being new with me constitutes the essence of my improvement. What has been hitherto known in the art as "tantalum," which occurs in the form of oxids or carbids of the metal, is an impure 25 amorphous powder not homogeneous and not ductile. Pure tantalum does not exist in nature in the state of a homogeneous ductile body. In fact, tantalum metal, as such, does not exist in the natural state at all. It 30 exists only in the condition of ores containing tantalum—such, as, for instance, in the columbite ore. Up to the present time it has been possible to extract from this ore an amorphous gray powder of tantalum only, or 35 a more or less coherent mass of impure tantalum which did not form in any way a homogeneous body and which was absolutely in- ductile. These tantalum compounds were useless for technical purposes.

40 I have discovered that by suitably treating the amorphous powders or tantalum compounds in the way, for example, as described in my prior application, Serial No. 187,830, filed in the United States Patent Office, Janu- 45 ary 5, 1904, of which the present application is a division, there may be produced a homogeneous ductile body highly refractory which has a melting-point at above 2,000° Celsius. This new metal I call substantially "pure 50 metallic tantalum," and it is distinguished from the impure products formerly known as "tantalum," as above indicated by possess-

ing the qualities of ductility and homogeneousness, while the impure compounds are brittle and non-homogeneous.

In order to produce this new metal, I subject the powder of the metal to be treated to sufficient pressure to practically bind or unite it together or to give to it a coherent or relatively solid mass and then pass a current of 60 electricity through it, preferably while it is submerged in a rare atmosphere approximating a vacuum. For best effecting this the mass of compressed powder is secured between clamps of tantalum constituting the 65 terminals of a source of electrical energy.

The metal commences to fuse as soon as an electrical current of sufficient intensity is led through the compressed powder. The fusing process will generally proceed with relation to such compressed body of powder upon the principle that a small bar fuses at its thinnest point, or at the point of smallest cross-section, and hence highest resistance. An arc is therefore formed at the fusing-point, 75 and in this arc the further parts of the bar melt down, so that more or less large beads of molten metal collect at the molten ends. These beads drop off as the fusing proceeds.

The small bars of compressed metal powder are placed on a plate of very refractory metal—for instance, of tantalum which forms one electrode—the other electrode being then approached to this body of compressed metal powder until both come into contact with 85 each other. Thereupon the other electrode is somewhat removed again, whereby an arc is formed in which the body of metal powder gradually melts. The molten body remains on the plate. It is also possible, of course, to 90 place a crucible below the arc and allow the molten metal to go on dropping into it as the fusing proceeds.

If the molten metal is brought into contact during the fusing process with other substances with which it is very liable to combine chemically at high temperatures, the result will be a strongly impure product and, as almost all very refractory metals are most apt to chemically combine with other substances at the high temperatures here in question, it is extremely difficult to obtain a pure metal. Above all, no carbon must be used as an electrode for fusing the metal, as

otherwise the metal would take up too much carbon and might under circumstances be changed into a carbid. Further, all oxygen must be kept away, and therefore all air must

5 be pumped out of the fusing vessel as far as possible. Tantalum metal and many others are also liable to chemically combine with nitrogen, hydrogen, &c., and consequently these injurious gases must also be kept away.

10 Therefore I prefer to execute the fusing process in a vacuum as perfect as can be obtained and to have the electrodes between which the fusing takes place out of the same metal as that which is to be fused.

15 I have found that it is best to use direct current for the fusing process and to bring the metal to be fused into contact with the positive electrode. This electrode may consist, for instance, of a small plate of the same

20 metal as that which is to be fused. The negative electrode may consist of another metal,

as it will not so easily be brought to fusing.

25 The metallic body formed according to this process is quite homogeneous and has a very high degree of ductility. Thus it is possible without difficulty to produce quite homogeneous bodies of tantalum metal. If pure raw material is used for the purpose and if all impurities are kept away during that fusing

30 process, the tantalum metal so obtained will have such a high degree of ductility that it can be rolled into very fine sheets and drawn into the finest of wires, while formerly it was generally thought that pure tantalum metal

35 was quite brittle and could in no way be worked mechanically.

It will be apparent that the new metal having the characteristics described will have a wide use in the arts.

I make no claim hereinafter to the method or process hereinbefore described, as this constitutes the subject-matter of the before-mentioned original application, my claims in the present instance being directed generically to the product which results from such process, there not having been known in the art of metallurgy, prior to my invention, in so far as I am aware, a product of the highly-refractory metal hereinbefore named other than in the nature of an impure metal powder of non-homogeneous character which could not, as hereinbefore stated, be utilized in the arts for the purpose of making such highly-refractory metals possessing the qualifications of homogeneity and ductility.

Having thus described my invention, what I claim as new, and desire to secure by Letters Patent, is—

1. A metal derived from tantalum compounds and possessing the quality of being homogeneous and ductile.

2. Substantially pure metallic tantalum possessing the qualifications of homogeneity and ductility.

In testimony whereof I have signed my name to this specification in the presence of two subscribing witnesses.

WERNER VON BOLTON.

Witnesses:

HENRY HASPER,  
WOLDEMAR HAUPT.